

## 1

3,666,545

### METHOD OF PRODUCING AN OPAQUE, LIGHT WEIGHT FABRIC AND RESULTANT FABRIC

John A. Pinatel, P.O. Box 490, Joliette, Quebec, Canada, and Georges A. Pascall, Montreal, Quebec, Canada; said Pascall assignor to said Pinatel

No Drawing. Filed July 15, 1969, Ser. No. 842,010  
Claims priority, application Canada, July 26, 1968,  
026,094

Int. Cl. B32b 27/36, 27/20

U.S. Cl. 117—138.8 F

4 Claims

#### ABSTRACT OF THE DISCLOSURE

A light weight spunbonded polyester fabric having a weight of about 1.2 to 1.4 oz./yd.<sup>2</sup> has applied thereto a very thin film of opaquesing material consisting of a self-crosslinking acrylic emulsion polymer of a colloidal dispersion of a vinyl chloride or a polysiloxane containing 20 to 30% by weight of an opaquesing filler. About 1 oz. of dry opaquesing solids is applied per square yard of fabric.

#### BACKGROUND OF THE INVENTION

##### (1) Field of the invention

This invention relates to a method of treating light weight non-woven fabrics to provide opacity and to the fabrics so treated.

##### (2) Description of prior art

Non-woven fabrics, such as spunbonded polyesters, have come into wide spread use because of their many unique properties. Thus, very light weight spunbonded fabrics have high tensile strength, excellent tear strength, non-raveling edges and superior dimensional stability. Because of such qualities they are widely used as apparel interliners, labels, base fabrics for books and wallcoverings, bags, electrical laminates and backings for leather or vinyl coated shoe linings.

Another interesting feature of non-woven fabrics is that they are very inexpensive to produce so that they show great promise for use as disposable articles. The main disadvantage of light weight non-woven fabrics is that they tend to be transparent, or at least translucent, and this greatly restricts the number and variety of their possible uses as disposable articles, e.g. for disposable garments, sheets, etc.

It is an object of this invention to provide a low cost method of opaquesing such light weight non-woven fabrics.

#### SUMMARY OF THE INVENTION

According to our invention a light weight, non-woven fabric has applied thereto a very thin layer of an opaquesing material comprising a fabric treating polymer emulsion or dispersion containing about 20 to 30% of an opaquesing filler.

Among suitable fabrics to be treated there can be mentioned rayon, acetate, nylon and polyester. Spunbonded polyester fabrics made from crimped fibers have been found to be particularly suitable for articles of apparel and bed sheets because of their soft, comfortable hand. In order to keep the fabric cost as low as possible,

## 2

a very light weight fabric should be used, e.g. one weighing about 1.2-1.4 oz./yd.<sup>2</sup>.

Almost any polymeric emulsion or dispersion which is available for treating fabrics of the above types can be used according to our invention. It is, of course, desirable to use polymers which have a very high curing rate at a low curing temperature. The high curing rate is important for low production costs, while some of the fabrics may contain heat sensitive fibers making low curing temperatures important.

Among suitable polymeric materials there can be mentioned colloidal dispersions of vinyl chloride polymers and copolymers in water and acrylic emulsion copolymers, particularly self-crosslinking acrylic polymers. Another polymer which can be used is a polysiloxane rubber which has the advantage of providing waterproofness to the fabric. These polymeric materials may or may not be preplasticized and if a separate plasticizer is necessary, this can be selected from a wide variety of commercially available agents.

It is particularly desirable to use plasticizers which will also impart flame resistance to the fabric, e.g. phosphates or antimonates. Tricresyl phosphate is a particularly good plasticizer which imparts to the fabric a durability against deterioration by washing and/or dry cleaning, while also imparting flame resistance. Another highly suitable plasticizer is a mixture of tri- and di-chloropropyl phosphate, which can be used together with di-ammonium phosphate to provide flame-proofing.

A wide variety of opaquesing fillers can be used according to our invention. These include, inter alia, any one of, or any mutually compatible combination of, the following substances

- 35 (1) Talc
- (2) A superflos
- (3) Clay
- (4) Flocks or powders of natural or synthetic fibers.

40 The superflos is a carbonate of silicon, magnesium aluminum or calcium and is available in the form of a very light powder having a very high covering power. Mixtures of such substances appear in the natural state, for example, in the mineral wollastonite.

45 As flocks or powders of natural or synthetic fibers there can be used flocks or powders of cellulosic fibers including cotton and rayon fibers or acrylic fibers.

The fillers may also contain additional ingredients including extenders, dispersing agent and pigments.

50 Among suitable extenders there can be mentioned a synthetic silicate, for example, a hydrous calcium silicate produced by the hydrothermal reaction of diatomaceous silica and lime or magnesium. The extender is chosen with the view to the subsequent treatment to which the fabric is to be exposed. For example, if it is to be subjected to a form of printing that uses a water based colouring, then a grade of extender is selected having a high water absorption (e.g. 500% or more), whereas, if an oil based printing step is followed, a grade of extender is selected having a high oil absorption (e.g. also about 500%). The extender then acts to suck up and firmly hold the colouring matter and thus gives the finished product a bright, fully coloured appearance.

As dispersing agents, organic dispersants can be used as well as inorganic agents, such as potassium tetraphosphate.

The pigments can be selected freely depending on the desired finish of the fabric. If the fabric is to be white, a rutile grade of titanium dioxide may be used, while if a shiny or silk-like surface is desired a synthetic pearl pigment, such as guanine, can be used. When the filler contains acrylic flocks, particularly vibrant colours can be obtained with cationic dyes.

A thin film of most of the opaques can best be applied by means of a roller, such as an engraved roller, or kiss roller or by means of a doctor blade. For this type of application the opaques must be reasonably viscous, e.g. 7,000 and higher Brookfield viscosity, and this may require the addition of a thickener. Among very satisfactory thickeners there can be mentioned hydroxyethyl cellulose.

After the film has been applied, the fabric is dried by passing it over calender rolls and through a drying chamber at temperatures up to about 300° F.

It is an important feature of the invention that a very thin and even layer of opaques be applied to the fabric. This is important both for manufacturing costs and the softness of the finished fabric. Generally only about 1-2 ounces of opaques dry solids are applied per square yard of fabric and about 1-1.5 ounces are particularly desirable.

When the fabric is being coated with a polysiloxane rubber containing fillers, this can successfully be applied from a relatively thin solution in a padding bath. The fabric treated in this manner is dried in a conventional pin stander at a temperature of up to 300° F. The polysiloxane treated fabric is waterproof and is particularly useful for making disposable sheets for hospital beds.

#### Working examples

The invention is illustrated by the following working examples:

##### EXAMPLE 1

An opaque composition was prepared having the following ingredients, all percentages being by weight.

|                                                                                                                       | Percent |
|-----------------------------------------------------------------------------------------------------------------------|---------|
| Polyvinyl chloride latex (Geon)                                                                                       | 40      |
| Tricresyl phosphate                                                                                                   | 10      |
| Filler—mixture of 10% talc, 12% superflos and 3% extender plus a small amount of tetraphosphate as a dispersing agent | 25      |
| Hydroxyethyl cellulose                                                                                                | 1-5     |
| Water, balance to 100%.                                                                                               |         |

This composition was then used to provide opaques to a spunbonded polyester fabric available under the trademark Reemay. The fabric had a thickness of 10 mils and a weight of 1.2 oz./yd.<sup>2</sup>.

The opaque composition was applied to the fabric by means of an engraved roller at room temperature and a fabric speed of 50 yd./min. The treated fabric was dried by passing over calender rolls and through a hot chamber for 3 minutes at temperatures up to 300° F. About 1.1 oz. of dry solids were deposited per square yard of fabric.

The finished fabric showed excellent opacity and was readily dyeable to any desired colour.

##### EXAMPLE 2

An opaque composition was prepared having the following ingredients, all percentages being by weight:

|                                                                                                                              | Percent |
|------------------------------------------------------------------------------------------------------------------------------|---------|
| Self-crosslinking acrylic polymer (Rhoplex HA-8)                                                                             | 50      |
| Tri- and di-chloropropyl phosphate                                                                                           | 7       |
| Filler-mixture of 20% superflos, 3% talc and 2% extender plus small amount of potassium tetraphosphate as a dispersing agent | 25      |
| Hydroxyethyl cellulose                                                                                                       | 1       |
| Oil and water repellent (Scotchgard 212 FC)                                                                                  | 2-4     |
| Liquid ammonia to adjust pH to 8                                                                                             | Trace   |
| Water, balance to 100%.                                                                                                      |         |

This composition was also used to coat Reemay fabric under the same conditions as in Example 1. Again excellent opacity was obtained.

##### EXAMPLE 3

Another opaque composition was prepared having the following ingredients:

|                        | Lbs. |
|------------------------|------|
| Water                  | 50   |
| Talc                   | 25   |
| Superflos              | 10   |
| Hydroxyethyl cellulose | 1    |
| Rhoplex HA-8           | 30   |
| Tricresylphosphate     | 5    |

The batch was made up to 10 Imperial gallons and the pH was adjusted to 8 with ammonia.

Reemay fabric was coated with the above composition under the same conditions as in Example 1 and once again excellent opacity was obtained.

##### EXAMPLE 4

An opaque composition was prepared having the following ingredients, all percentages being by weight:

|                                                     | Percent |
|-----------------------------------------------------|---------|
| Water                                               | 43.0    |
| Cellulose fibre powder                              | 25.0    |
| Acrylic polymer (experimental emulsion E-485)       | 30.0    |
| Sodium salt of carboxylated polyelectrolyte (Tomol) | 0.2     |
| Hydroxyethyl cellulose                              | 1.8     |
|                                                     | 100.0   |

The pH was adjusted to 8 with ammonia and the composition was used to treat Reemay according to the procedure of Example 1. Excellent opacity was obtained.

##### EXAMPLE 5

An opaque composition was prepared having the following ingredients, all percentages being by weight:

|                                                    | Percent |
|----------------------------------------------------|---------|
| Dimethyl polysiloxane (Dow Corning 236 dispersion) | 35      |
| TiO <sub>2</sub>                                   | 20      |
| Organic solvent, balance.                          |         |

This composition was applied to Reemay fabric by passing the fabric through a padding bath. The wet chemical pick-up was about 40% and the treated fabric was dried in a conventional pin stander at temperatures up to 300° F.

The dried, treated fabric was not only opaque but was also waterproof, making it excellent material for disposable hospital sheeting.

We claim:

1. A method of producing an opaque, light weight, disposable fabric which comprises applying to a spunbonded polyester fabric having a weight of 1.2 to 1.4 oz./yd.<sup>2</sup> a thin layer of an opaque composition comprising a polymeric emulsion or dispersion selected from the group consisting of a colloidal dispersion of vinyl chloride polymers, acrylic emulsion polymers and polysiloxanes containing 20-30% by weight of opaque filler, the opaque composition having a Brookfield viscosity of about 7000 to 8000 and being applied by means of an engraved roller, and drying the coated fabric to provide a layer of about 1-2 ounces of dry solids per square yard of fabric.

2. An opaque, spunbonded polyester fabric obtained by the method of claim 1.

3. A method of producing an opaque, light weight, disposable fabric which comprises applying to a spunbonded polyester fabric having a weight of 1.2 to 1.4 oz./yd.<sup>2</sup> a thin layer of an opaque composition comprising a self-crosslinking acrylic fabric treating polymer containing

20-30% by weight of opaques filler, the opaques composition having a Brookfield viscosity of about 7000 to 8000 and being applied by means of an engraved roller, and drying the coated fabric to provide a layer of about 1-1.5 ounces of dry solids per square yard of fabric. 5

4. A method of producing an opaque, light weight, disposable fabric which comprises applying to a spunbonded polyester fabric having a weight of 1.2 to 1.4 oz./yd.<sup>2</sup> a thin layer of an opaques composition comprising a fabric treating colloidal water dispersion of vinyl chloride copolymer containing 20-30% by weight of opaques fillers, the opaques composition having a Brookfield viscosity of about 7000 to 8000 and being applied by means of an engraved roller, and drying the coated fabric to provide a layer of about 1-1.5 ounces of dry solids per 10 square yard of fabric. 15

## References Cited

## UNITED STATES PATENTS

|           |         |                 |       |             |
|-----------|---------|-----------------|-------|-------------|
| 2,626,941 | 1/1953  | Habeck          | ----- | 260—41 A    |
| 2,881,146 | 4/1959  | Remer et al.    | ----- | 117—139.5 A |
| 3,077,460 | 2/1963  | Fortess         | ----- | 117—139.5 A |
| 3,248,314 | 4/1966  | Nahin           | ----- | 260—41 A    |
| 3,009,822 | 11/1961 | Drellich et al. | ----- | 117—38      |
| 3,228,790 | 1/1966  | Sexsmith et al. | ----- | 117—38 X    |
| 3,274,018 | 9/1966  | Russell et al.  | ----- | 117—38 X    |

RALPH HUSACK, Primary Examiner

U.S. Cl. X.R.

117—38, 136, 138.8 N, 139.5 A, 140 A, 145, 161 UC, 15 2 A, UF; 161—6